

Patented Nov. 2, 1926.

1,605,649

# UNITED STATES PATENT OFFICE.

ERNEST B. CURTIS, OF BROOKLYN, NEW YORK, ASSIGNOR TO AMERICAN RUBBER COMPANY, OF EAST CAMBRIDGE, MASSACHUSETTS, A CORPORATION OF MASSACHUSETTS.

## PROCESS OF TREATING FABRIC AND ARTICLE PRODUCED.

No Drawing.

Application filed July 17, 1923. Serial No. 652,203.

This invention relates to a process of treating fabrics and to the article produced, more particularly to a process for treating material such as haircloth to prevent raveling thereof and to the article produced thereby.

For many years a woven fabric known as haircloth has been produced, which is made by weaving the relatively stiff and coarse hairs obtained from the tails and manes of horses and from cattle, and such cloth has come into extensive use by tailors as a stiffening material in clothing to assist it in retaining its shape. The cloth commonly used for this purpose is not formed entirely of hair, but is made with warp threads of cotton or similar material, while the filler threads are composed of hair. A serious objection to the use of such material in clothing is that owing to the stiffness, coarseness and gloss of the hair it is not strongly held in its woven condition, but tends to work out or unravel. The ends of such loose hairs coming in contact with the body of the wearer are very uncomfortable, while if they work out to the exterior of the article of clothing its appearance is injured. It is my belief that attempts have been made to prevent this unraveling by coating the hair cloth with some form of sizing material or with unvulcanized rubber cement or balata. Such sizing, however, is relatively stiff and inflexible and cracks during wear, and if the article is subjected to steaming or wet cleaning the size dissolves. Hence the hair in the hair cloth treated in this manner tends to work out in the same way as with untreated haircloth. In the case of haircloth treated with unvulcanized rubber cement or balata these materials are soluble in the powerful solvents, such as carbon tetrachloride and gasoline, which are used for dry cleaning purposes. As a result after one or two dry cleanings haircloth treated in this manner also tends to unravel, causing the garment to lose its proper shape.

An object of my invention is to provide an improved process for treating haircloth and similar materials which permanently prevents unraveling in use.

Another object is to provide a haircloth having a binder incorporated therein which will be unaffected by use or cleaning.

For a detailed disclosure of the invention reference is had to the accompanying specification and claims.

In carrying out my invention haircloth, either that formed entirely or partially of hair, is impregnated with a material which after deposition in and on the fabric is insoluble in the ordinary solvents or materials used for cleaning clothing. In one example the haircloth may be impregnated, as by dipping, spraying or in any other suitable manner, with rubber latex and the fabric then dried. Rubber latex, owing to its fluidity, readily penetrates between the individual fibres composing the fabric and binds them firmly together, so that when in use it is impossible for the hair to unravel. As is well known ordinary rubber cement is made from rubber which has been milled or broken down, and the solution obtained by dissolving such rubber in an organic solvent contains a relatively small percentage of rubber, and does not readily penetrate into the fibres of a fabric, so that the latter cannot be as thoroughly impregnated as in the case of rubber latex. The most important respect, however, in which the latex treated haircloth is superior is that the natural latex rubber contained therein is in an unmilled or unbroken down condition and is therefore not readily soluble in the ordinary rubber solvents. For instance a sample of hair cloth which had been soaked for fifteen minutes in rubber latex containing about 35% rubber solids and dried was found to be practically unaffected after soaking for eighteen hours in carbon tetrachloride, and the hairs of the fabric were still firmly held in position.

If desired the rubber impregnated haircloth may be vulcanized, provided the vulcanization is effected at a temperature low enough to prevent injury to the hair. As an example a piece of haircloth may be immersed in rubber latex of 25% rubber solids and containing curing ingredients embodying low temperature curing accelerators. After drying the cloth may be allowed to cure at ordinary temperatures, or the cure may be hastened by heat, but the temperature should not be raised to such a point as to injure the hair, and it has been found that temperatures from 150° to 200° F. are suitable. One means of carrying out the above

is to employ latex which contains 1 part of zinc dimethyldithiocarbamate, 1 part of zinc oxide and 3 parts of sulphur on 100 parts of rubber. Haircloth impregnated 5 with this mixture and dried will vulcanize satisfactorily overnight at 150° F. or in 2 hours at 200° F. A sample of haircloth treated in this manner was also soaked in carbon tetrachloride for eighteen hours, at 10 the end of which time the hairs were still firmly fixed in place.

Instead of using rubber latex the hair cloth may be impregnated with one of the so-called "cold cure cements", the solvent 15 allowed to evaporate, and vulcanization secured with or without elevating the temperature. One means of accomplishing this is to treat the haircloth with rubber cement containing 100 parts of rubber, 20 parts of 20 zinc oxide, 3 parts of zinc butyl xanthogenate 1½ parts of dibenzylamine and 3 parts of sulphur, which after evaporation of the solvent will vulcanize satisfactorily in 48 hours at room temperature or in 30 minutes 25 at 200° F. A sample of material treated in this manner was soaked in carbon tetrachloride for four hours, when it was found that the hairs were still firmly fixed in place. Another means for accomplishing the same 30 result is to impregnate the haircloth with rubber cement containing 100 parts of rubber, 20 parts of zinc oxide, 3 parts of dibenzylamine, 3 parts of sulphur. After the solvent has dried out the treated haircloth is 35 painted with carbon disulphide. Thereafter the rubber will cure in 48 hours at ordinary temperatures or in 60 minutes at 200° F. It is preferred, however, to use latex for the impregnation owing to its greater 40 penetrative power, its insolubility after coagulation, its strength, and the firm union between it and the fibres. It is also obvious that if desired the material may be vulcanized by the well known cold cure method, 45 using sulphur monochloride in liquid or gaseous form. In still another modification, the material may be impregnated by the use of a solution of vulcanized rubber, and the solvent driven off, leaving a deposit of vulcanized rubber in the haircloth.

Haircloth treated according to the invention is especially adapted for use by tailors,

not only by reason of the fact that the hairs cannot unravel either in use or after any of the ordinary forms of cleaning, but also due 55 to the fact that the rubber impregnation increases the tensile strength, elasticity and body of the material without the loss of any necessary flexibility. It is obvious that the process is not limited in its application to 60 haircloth, but it may also be used in any case where the threads of a fabric are composed of any material tending to unravel or disintegrate in a similar manner.

While the invention has been described in 65 detail it is obvious that numerous modifications will suggest themselves to those skilled in the art, and it is not desired that it be limited otherwise than as set forth in the appended claims.

Having thus described my invention, what I claim and desire to protect by Letters Patent is:—

1. The process of proofing haircloth against raveling which comprises impregnating it with a fluid containing a flexible rubber containing binder relatively insoluble in rubber solvents after deposition, and removing the fluid contents to deposit the binder in the haircloth. 75

2. The process of proofing haircloth against raveling which comprises impregnating it with rubber latex, and drying, and allowing it to vulcanize at temperatures not injurious to the haircloth. 80

3. As a new article of manufacture, a woven haircloth having the individual fibres thereof held against slipping by a binder of the solid constituents of rubber latex relatively insoluble in rubber solvents. 85

4. As a new article of manufacture a haircloth impregnated with dried latex rubber. 90

5. As a new article of manufacture a haircloth impregnated with vulcanized latex rubber. 95

6. As a new article of manufacture a haircloth impregnated with a low temperature vulcanized latex rubber.

Signed at New York, county of New York, and State of New York, this 13 day of July, 1923.

ERNEST B. CURTIS.